

L. S. BACHE.  
SELF LUBRICATING WOOD BEARING AND SURFACE.  
APPLICATION FILED JULY 6, 1911.

1,076,941.

Patented Oct. 28, 1913.

FIG. 1.



FIG. 2.



WITNESSES:

J. G. D. Bache  
R. A. Brenner

INVENTOR

Leigh S. Bache  
BY  
C. A. Baker  
ATTORNEY

# UNITED STATES PATENT OFFICE.

LEIGH S. BACHE, OF BOUND BROOK, NEW JERSEY, ASSIGNOR TO GRAPHITE LUBRICATION COMPANY, OF BOUND BROOK, NEW JERSEY, A CORPORATION OF NEW JERSEY.

## SELF-LUBRICATING WOOD BEARING AND SURFACE.

1,076,941.

Specification of Letters Patent.

Patented Oct. 28, 1913.

Application filed July 6, 1911. Serial No. 637,206.

To all whom it may concern:

Be it known that I, LEIGH S. BACHE, a citizen of the United States, and a resident of Boundbrook, in the county of Somerset 5 and State of New Jersey, have invented certain new and useful Self-Lubricating Wood Bearings and Surfaces, of which the following is a specification:

The invention relates to a bearing or bearing surfaces of wood, the material being so treated that it is absolutely self-lubricating and will retain its lubrication.

The object of the invention is to produce a wood bearing of any desired form so treated that it will maintain a lubricating surface, be practically non-destructible as against wear and will retain its lubricating features under all conditions of use.

Referring to the drawings: Figure 1 illustrates a block of wood of improper character, the imperfection showing during treatment. Fig. 2 illustrates a block of wood of perfect character after treatment. Fig. 3 is a sectional view illustrative of an imperfectly treated wood bearing. Fig. 4 is illustrative of a perfectly treated wood bearing.

It is not new in the art to treat wood and fiber with water-proofing and lubricating materials which give a greater or less permeating effect; nor is it new to stain wood and fiber either with or without a water-resisting filler. The invention herein defined goes further than the mere staining or surface-lubrication of wood or fiber and contemplates a new field in which the material to be used is completely, regularly and absolutely permeated by the impregnating substance which, as hereinafter described, is bound in the fiber so that there is a complete and efficient lubrication at all times without liability of dissipation of the impregnating material at certain parts of the structure.

The process under which the bearings or bearing surfaces are treated is fully described in a co-pending application, Serial No. 637,207, filed July 6, 1911, entitled Process of treating and coloring wood, and the process *per se* forms no part of the present application, which is confined to an article of manufacture, namely, a bearing of wood which is self-lubricating, non-impermeous to moisture, and has wearing qualities to almost unlimited capacity.

In producing the bearings a suitable block 55 of substantially dry wood or fiber of analog-

ous character is utilized and this block of wood or fiber is subjected to treatment in a boiling mass of saturated hydro-carbon, such as paraffin, a wax, and oxidized hydro-carbon having a low melting point, such as 60 rosin, through which mixture is infused a coloring matter preferably such as is soluble in oil, as for instance, a coloring matter having an indulin base made soluble with stearin and olein. In some treatments stearic 65 acid is also used in the bath. The wood or fiber is boiled in this bath until its gravity is such that it falls to the bottom of the receptacle, this being the best indication that it is thoroughly impregnated. There is a 70 particular advantage in subjecting the material to be treated to the bath having as an element the coloring matter. This is illustrated in the drawings.

In Fig. 1, there is shown a block of 75 wood or analogous fiber *a*, having streaks *b*, of various proportions extending along or through the wood. These streaks are due to "tight-grain," "dry-rot," or "sap-grain" which ordinarily would not appear in the 80 material and would not be discernible in using the wood in the ordinary arts of manufacture. When such a block is submitted to treatment, the streaking indicated by the letter *b*, is prominently shown in light colors. The impregnating materials do not carry through in these streaks, and as the impregnating material acts as a conveyer for the coloring matter, such portions are uncolored and readily indicate whether or not 90 the block of wood or fiber is suitable for use.

Fig. 2 illustrates a block of wood or fiber *c*, which has no checks, "tight-grain," "dry-rot" or "sap-grain" and shows a perfect material suitable for bearings, shuttles or 95 like devices wherein an even and perfect filling and lubrication of the material is most essential.

In the bearings herein described, there is a permanency of homogeneous lubrication 100 apparently due to the binding effect of the coloring matter with reference to the impregnating materials.

In Fig. 3 there is well illustrated this feature of uneven distribution of the lubricant. Fig. 3 illustrates a sectional view of a straight line bearing treated merely with an impregnating oil and illustrating the drying out of the oil at the central portion *e*, and the excess lubrication at the ends *e'*, *e''*. 110

It has been found that practically all wood bearings treated with a lubricant under methods heretofore known, act as illustrated in Fig. 3. In fact, the oil or grease of the impregnating material boils out at the ends of the bearing leaving the center comparatively dry.

In Fig. 4 there is illustrated a sectional bearing *f*, treated as herein described, where-  
10 in there is a homogeneous and complete saturation of the material with the lubricant which is so bound by the coloring matter that there is no dissipation at any given point. Such a bearing will run with com-  
15 paratively no wear and for an indefinite period inasmuch as it is perfectly lubri- cated throughout its entire fiber. Furthermore it may be treated as a homogeneous piece of metal and when bored and finished  
20 will be in absolute balance.

It will be seen from the above that self-lubricating bearings produced as described may be made in perfect form and balance and that there is no waste in using materials  
25 of an imperfect character such as illustrated in Fig. 1.

In carrying out the invention the wood or fiber of any suitable form is subjected to a boiling bath of the materials indicated until  
30 thoroughly impregnated and is thereupon formed to provide any desired bearing. The ingredients of the bath may be varied to a considerable extent although excellent re- sults have been attained with a mixture sub-  
35 stantially as follows: paraffin 100 lbs., car- nauba wax 20 lbs., rosin, 20 lbs., coloring matter  $3\frac{1}{2}$  lbs., using in some instances a comparatively small portion by weight of stearic acid. It is a peculiarity of the treat-  
40 ment that, without the coloring matter, it is impossible to ascertain whether or not the material is properly impregnated. With the coloring matter, however, the material im- mediately shows, after treatment, the streak-

ing illustrated in Fig. 1 (denoting improper 45 impregnation) or the perfect form of Fig. 2.

The advantages are apparent inasmuch as with the given material, the fine work and expensive labor necessary to work the material into finished form need only be ex- pended upon suitable materials for produc-  
50 ing perfect goods. Furthermore, the ma- terial will be evenly and perfectly filled through and through and will produce arti- cles in perfect balance.

Obviously, the material may be worked into many forms other than the bearings of cylindrical form herein described and, in fact, may be used wherever a self-lubricat-  
55 ing material is required.

What I claim as my invention and desire to secure by Letters Patent is:

1. As an article of manufacture, a lubri- cated bearing of wood or the like impreg-  
60 nated through and through with a saturated hydro-carbon, wax, oxidized hydro-carbon and a coloring matter.

2. As an article of manufacture a lubri- cated bearing of wood or fiber impregnated through and through by subjecting to a hot  
70 bath containing saturated hydro-carbon, wax, oxidized hydro-carbon and a coloring matter.

3. As an article of manufacture a lubri- cated bearing of wood or fiber impregnated  
75 through and through by subjecting to a hot bath containing saturated hydro-carbon, wax, oxidized hydro-carbon, stearic acid and a coloring matter.

4. As an article of manufacture, a lubri-  
80 cated bearing of wood or the like impreg- nated through and through with a saturated hydro-carbon, wax, oxidized hydro-carbon, stearic acid and a coloring matter.

LEIGH S. BACHE.

Witnesses:

A. LANG,  
GEO. O. SMALLEY.